

## UNITED STATES PATENT OFFICE

2,035,415

## ALLOY

Richard A. Wilkins, Rome, N. Y., assignor to  
 Revere Copper and Brass Incorporated, Rome,  
 N. Y., a corporation of Maryland

No Drawing. Application March 2, 1935,  
 Serial No. 9,111

4 Claims. (Cl. 75—1)

My invention relates to alloys.

Applicant has found that ternary copper-silicon-tin alloys with a high copper content and the silicon and tin within certain ranges and proportions possess a high resistance to corrosion, a high tensile strength, and relatively high ductility or elongation in both the fully annealed and cold worked conditions, and that they may be heat treated when cold worked markedly to increase their yield point without reduction or marked change in tensile strength, ductility and hardness.

It has been found that if iron is added to these alloys the hardness may be controlled both by varying the amount of iron and by heat treatment of the alloy without materially decreasing the resistance to corrosion or other properties of the alloy except a slight increase in tensile strength at the expense of a slight decrease in ductility.

Preferably the amount of iron is such in relation to the amount of silicon as to cause all the iron to be in the form of iron silicide, thus avoiding the presence of free iron which otherwise would be present due to the insolubility of the iron in the copper-base. Any deleterious effect on the corrosion resistance of the alloy due to the presence of iron silicide and minute quantities of free iron is more than offset by the tin. The iron silicide it has been found apparently dissolves in the fully annealed alloy, but precipitates in the heat treated alloy to form needle-like crystals which act to lock together the glide planes of the crystals of the basic alloy. Thus in the fully annealed alloy the hardness is not materially affected by the addition of iron to the basic alloy, but in the heat treated alloy the addition of iron secures a noticeable hardening effect.

Under some conditions of use it may be desirable to increase the hot working properties of the alloy. It has been found that this conveniently may be done by adding zinc. Preferably the amount of zinc should not exceed about 2% where the alloys are to be used for welding purposes, but otherwise the amount of zinc may be such that the sum of the silicon, tin, iron and zinc does not exceed about 10%. In other words, a maximum of about 7.65% zinc may be employed when the alloy contains the minimum values hereinafter specified of silicon, tin and iron. As little as 0.1% zinc under many conditions will secure noticeable results.

The zinc by improving the hot working properties of the alloy enables many mill products to be fabricated more easily of the alloy, and in

some instances is further desirable to control the hardness, tensile strength and ductility of the alloy. Silicon tends to increase the tensile strength at the expense of the ductility, as likewise does iron, the latter also acting as a hardener. Tin in conjunction with silicon acts to increase both the tensile strength and ductility, as compared to a binary copper-silicon alloy. Zinc acts to increase the ductility at the expense of the tensile strength and hardness. Therefore zinc when properly proportioned to the silicon, tin and iron acts to control the tensile strength, ductility and hardness.

In the improved alloy, although the preferred range of silicon is approximately 2.75 to 3.5%, below which range the tensile strength and yield point increasingly decrease and above which range the alloy becomes increasingly difficult to cold work, the silicon in many instances may be as low as 2% and as high as 4.5% and still an alloy be secured which commercially has the desired properties.

The alloy in respect to many of its properties is rather sensitive to iron, and ordinarily the latter should be maintained between approximately 0.1 and 0.6% so as not deleteriously to affect the properties of the alloy. A preferred value of 0.25% iron ordinarily gives excellent results.

The preferred range of tin for the above mentioned preferred range of silicon is 0.25 to 0.5%, but by maintaining a proper relation between the tin and silicon the amount of tin in some instances may be materially increased. As little as 0.25% tin may be present for all values of silicon from 2 to 4.5%, above which range it is impossible economically to cold work the alloy no matter what the amount of tin or zinc. But to maintain the alloy hot workable within this range of silicon the tin should not exceed roughly 2% for all values of silicon up to 3%, and for any value of silicon above 3% should not exceed a value roughly represented by a linear decrease in tin from 2% at 3% silicon to 1.7% at 3.5% silicon and to 1.1% at 4.5% silicon.

The alloys according to the invention may be fully annealed by heating them to about 1200 to 1300° F. Within the preferred ranges of 2.75 to 3.5% silicon, 0.25 to 0.5% tin, 0.25% iron, and up to 2% zinc, all the alloys will have a tensile strength of at least approximately 55,000 pounds per square inch and an elongation of at least approximately 65% in two inches. All the alloys are capable of being cold drawn into rods having a tensile strength of at least approximately 55

105,000 pounds per square inch and an elongation of at least approximately 10% in two inches, and are capable of being cold rolled into sheets having a tensile strength of at least approximately 100,000 pounds per square inch and an elongation of at least approximately 5% in two inches. In general the tensile strength will decrease and the ductility increase with the amount of zinc, as above explained, but in no instance will they go below the approximate values above given when the alloys are within the preferred ranges of constituents. All the alloys within the larger ranges above specified will have in the fully annealed condition a tensile strength of at least approximately 50,000 pounds per square inch and an elongation of at least approximately 60% in two inches, and all are capable of being cold drawn into rods having a tensile strength of at least approximately 100,000 pounds per square inch and an elongation of at least approximately 8% in two inches, and all are capable of being cold rolled into sheets having a tensile strength of at least approximately 90,000 pounds per square inch and an elongation of at least approximately 5% in two inches.

When fully annealed the alloys are capable of at least 50% reduction by cold rolling or drawing without again annealing them. This enables them readily to be cold worked into articles. By heating the cold worked articles to 500 to 600° F. for 30 to 90 minutes and cooling them in air at room temperature the yield point and hardness will be markedly increased without any material change in the tensile strength or elongation. It will be observed that this heat treatment is performed at temperatures below the full annealing temperatures, or, in other words, is performed at temperatures below the recrystallization temperatures of the copper-silicon-tin-zinc solution, although performed at the temperatures at which dissolved iron silicide will precipitate as has hereinbefore been referred to.

It will be understood that small amounts of metals other than those herein specified may be added to the alloys for imparting special characteristics when these metals do not destroy such valuable properties of the alloy as it may be desired to retain.

I claim:

1. Corrosion resistant copper base alloys capable of being worked both hot and cold containing copper, silicon, tin, zinc and iron within the following approximate ranges and proportions: silicon 2 to 4.5%, tin 0.25 to 2%, iron 0.1 to 0.6%, zinc appreciable amounts up to 7.65%, balance substantially all copper, the minimum amount of tin being 0.25% for all values of silicon, the maximum amount of tin being 2% for all values of silicon up to 3% and varying between 1.1 and 2% linearly and inversely with the amount of silicon when the latter is between 3 and 4.5%, and the sum of the silicon, tin, iron and zinc not exceeding 10%; the alloys being of relatively high tensile strength and ductility in both the fully annealed and cold worked conditions, and when cold worked from the fully annealed condition being capable of being heat treated for markedly increasing both the yield point and hardness with but relatively small change in the tensile strength and ductility.

2. Corrosion resistant copper base alloys capable of being worked both hot and cold containing copper, silicon, tin, zinc and iron within the following approximate ranges and proportions: silicon 2.75 to 3.5%, tin 0.25 to 2%, iron 0.1 to 0.6%, zinc appreciable amounts up to 2%, balance substantially all copper, the minimum amount of tin being 0.25% for all values of silicon, and the maximum amount of tin being 2% for all values of silicon up to 3% and varying between 1.7 and 2% linearly and inversely with the amount of silicon when the latter is between 3 and 3.5%; the alloys being of relatively high tensile strength and ductility in both the fully annealed and cold worked conditions, and when cold worked from the fully annealed condition being capable of being heat treated for markedly increasing both the yield point and hardness with but relatively small change in the tensile strength and ductility.

3. The alloys according to claim 2 having approximately 0.25 to 0.5% tin.

4. The alloys according to claim 2 having, approximately, 0.25 to 0.5% tin and 0.25% iron.

RICHARD A. WILKINS.